



US005206128A

# United States Patent [19]

Arai

[11] Patent Number: 5,206,128

[45] Date of Patent: Apr. 27, 1993

- [54] SILVER HALIDE PHOTOGRAPHIC MATERIAL

[75] Inventor: Naoki Arai, Kanagawa, Japan

[73] Assignee: Fuji Photo Film Co., Ltd., Kanagawa, Japan

[21] Appl. No.: 725,115

[22] Filed: Jul. 3, 1991

[30] Foreign Application Priority Data

Jul. 4, 1990 [JP] Japan ..... 2-176825

[51] Int. Cl.<sup>5</sup> ..... G03C 1/76

[52] U.S. Cl. ..... 430/539; 430/523;  
430/961

[58] Field of Search ..... 430/539, 525, 950, 961

[56] References Cited

U.S. PATENT DOCUMENTS

4,357,418 11/1982 Cellone ..... 430/539  
4,369,245 6/1983 Beruto et al. ..... 430/539  
4,399,213 8/1983 Watanabe et al. ..... 430/539

- |           |         |                      |         |
|-----------|---------|----------------------|---------|
| 4,450,230 | 5/1984  | Delfino et al. ....  | 430/539 |
| 4,455,365 | 6/1984  | Urata et al. ....    | 430/539 |
| 4,460,580 | 7/1984  | Ogawa et al. ....    | 430/639 |
| 4,476,218 | 10/1984 | Ogawa et al. ....    | 430/539 |
| 4,513,080 | 4/1985  | Helling ....         | 430/539 |
| 4,840,881 | 6/1989  | Watanabe et al. .... | 430/539 |
| 4,944,966 | 7/1990  | Jerenz ....          | 430/539 |

*Primary Examiner*—Jack P. Brammer  
*Attorney, Agent, or Firm*—Sughrue, Mion, Zinn,  
Macpeak & Seas

## ABSTRACT

A silver halide photographic material is described including a support having thereon an emulsion layer and a protective layer in this order, wherein gelatin is contained in the protective layer in an amount of at least 1.5 g/m<sup>2</sup>, gelatin is contained in the emulsion layer in an amount of at least 1.0 g/m<sup>2</sup>, and the total coated amount of gelatin in the protective layer and the emulsion layer is a total of at most 3.5 g/m<sup>2</sup>.

**4 Claims, No Drawings**

## SILVER HALIDE PHOTOGRAPHIC MATERIAL

## FIELD OF THE INVENTION

The present invention relates to a silver halide photographic material which can be processed by an ultrahigh speed automatic developing machine in a satisfactory manner. More particularly, the present invention relates to a silver halide photographic material which does not experience significant pinholing developed when the emulsion layer side of the silver halide photographic material is caught by small protrusions formed on the roller in the automatic developing machine during processing (hereinafter referred to as "scratch pinholing").

## BACKGROUND OF THE INVENTION

A light-sensitive material adapted for processing at an ultrahigh speed is subject to pinholing developed when the emulsion layer side of the light-sensitive material is caught by small protrusions formed on the surface of the roller in an automatic developing machine during processing.

## SUMMARY OF THE INVENTION

It is therefore an object of the present invention to provide a silver halide photographic material which is not susceptible to scratch pinholing, roller marking and underdrying, which can be easily developed in an ultrahigh speed automatic developing machine.

The above and other objects of the present invention will become more apparent from the following detailed description and examples.

The above object of the present invention is accomplished with a silver halide photographic material comprising a support having thereon at least one protective layer and at least one emulsion layer, wherein gelatin is contained in the protective layer in an amount of at least 1.5 g/m<sup>2</sup>, gelatin is contained in the emulsion layer in an amount of at least 1.0 g/m<sup>2</sup>, and the coated amount of gelatin in the protective layer and the emulsion layer is at most 3.5 g/m<sup>2</sup> in total.

## DETAILED DESCRIPTION OF THE INVENTION

The present invention is characterized by the distribution of the coated amount of gelatin. In particular, scratch pinholing, roller marking and the like are normally avoided by improving the gelatin film strength of the silver halide emulsion layer. To this end, the proportion of gelatin content to silver halide content in the emulsion, i.e., the coated amount of gelatin in the emulsion layer, is normally increased.

On the other hand, in order to provide a silver halide photographic material with adaptability to processing at an ultrahigh speed, the coated amount of gelatin is generally reduced uniformly in all gelatin-containing layers of the photographic material.

The present inventors have found that better adaptability to processing at an ultrahigh speed can be obtained by providing a particular distribution of the coated amount of gelatin between a protective layer and an emulsion layer, rather than by uniformly reducing the coated amount of gelatin in the protective layer and the emulsion layer as before.

In accordance with the present invention, the development of scratch pinholing and roller marking on a silver halide photographic material can be inhibited and

the dryability of the light-sensitive material can be improved in spite of a relatively small coated amount of gelatin in the emulsion layer by reducing the total coated amount of gelatin in the emulsion layer and the protective layer to 3.5 g/m<sup>2</sup> or less and increasing the coated amount of gelatin in the protective layer to 1.5 g/m<sup>2</sup> or more.

In the present invention, the silver halide emulsion layer may consist of two or more layers, and the protective layer includes all layers provided on the emulsion layer(s) (in the side further from the support) to protect the emulsion layer(s), such as a surface protective layer (outermost layer), a filter layer, an interlayer, an anti-  
10  
15  
16  
17  
18  
19  
20  
21  
22  
23  
24  
25  
26  
27  
28  
29  
30  
31  
32  
33  
34  
35  
36  
37  
38  
39  
40  
41  
42  
43  
44  
45  
46  
47  
48  
49  
50  
51  
52  
53  
54  
55  
56  
57  
58  
59  
60  
61  
62  
63  
64  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
339  
340  
341  
342  
343  
344  
345  
346  
347  
348  
349  
349  
350  
351  
352  
353  
354  
355  
356  
357  
358  
359  
359  
360  
361  
362  
363  
364  
365  
366  
367  
368  
369  
369  
370  
371  
372  
373  
374  
375  
376  
377  
378  
379  
379  
380  
381  
382  
383  
384  
385  
386  
387  
388  
389  
389  
390  
391  
392  
393  
394  
395  
396  
397  
398  
399  
400  
401  
402  
403  
404  
405  
406  
407  
408  
409  
409  
410  
411  
412  
413  
414  
415  
416  
417  
418  
419  
419  
420  
421  
422  
423  
424  
425  
426  
427  
428  
429  
429  
430  
431  
432  
433  
434  
435  
436  
437  
438  
439  
439  
440  
441  
442  
443  
444  
445  
446  
447  
448  
449  
449  
450  
451  
452  
453  
454  
455  
456  
457  
458  
459  
459  
460  
461  
462  
463  
464  
465  
466  
467  
468  
469  
469  
470  
471  
472  
473  
474  
475  
476  
477  
478  
479  
479  
480  
481  
482  
483  
484  
485  
486  
487  
488  
489  
489  
490  
491  
492  
493  
494  
495  
496  
497  
498  
499  
500  
501  
502  
503  
504  
505  
506  
507  
508  
509  
509  
510  
511  
512  
513  
514  
515  
516  
517  
518  
519  
519  
520  
521  
522  
523  
524  
525  
526  
527  
528  
529  
529  
530  
531  
532  
533  
534  
535  
536  
537  
538  
539  
539  
540  
541  
542  
543  
544  
545  
546  
547  
548  
549  
549  
550  
551  
552  
553  
554  
555  
556  
557  
558  
559  
559  
560  
561  
562  
563  
564  
565  
566  
567  
568  
569  
569  
570  
571  
572  
573  
574  
575  
576  
577  
578  
579  
579  
580  
581  
582  
583  
584  
585  
586  
587  
588  
589  
589  
590  
591  
592  
593  
594  
595  
596  
597  
598  
599  
599  
600  
601  
602  
603  
604  
605  
606  
607  
608  
609  
609  
610  
611  
612  
613  
614  
615  
616  
617  
618  
619  
619  
620  
621  
622  
623  
624  
625  
626  
627  
628  
629  
629  
630  
631  
632  
633  
634  
635  
636  
637  
638  
639  
639  
640  
641  
642  
643  
644  
645  
646  
647  
648  
649  
649  
650  
651  
652  
653  
654  
655  
656  
657  
658  
659  
659  
660  
661  
662  
663  
664  
665  
666  
667  
668  
669  
669  
670  
671  
672  
673  
674  
675  
676  
677  
678  
679  
679  
680  
681  
682  
683  
684  
685  
686  
687  
688  
689  
689  
690  
691  
692  
693  
694  
695  
696  
697  
698  
698  
699  
699  
700  
701  
702  
703  
704  
705  
706  
707  
708  
709  
709  
710  
711  
712  
713  
714  
715  
716  
717  
718  
719  
719  
720  
721  
722  
723  
724  
725  
726  
727  
728  
729  
729  
730  
731  
732  
733  
734  
735  
736  
737  
738  
739  
739  
740  
741  
742  
743  
744  
745  
746  
747  
748  
749  
749  
750  
751  
752  
753  
754  
755  
756  
757  
758  
759  
759  
760  
761  
762  
763  
764  
765  
766  
767  
768  
769  
769  
770  
771  
772  
773  
774  
775  
776  
777  
778  
779  
779  
780  
781  
782  
783  
784  
785  
786  
787  
788  
789  
789  
790  
791  
792  
793  
794  
795  
796  
797  
798  
799  
800  
801  
802  
803  
804  
805  
806  
807  
808  
809  
809  
810  
811  
812  
813  
814  
815  
816  
817  
818  
819  
819  
820  
821  
822  
823  
824  
825  
826  
827  
828  
829  
829  
830  
831  
832  
833  
834  
835  
836  
837  
838  
839  
839  
840  
841  
842  
843  
844  
845  
846  
847  
848  
849  
849  
850  
851  
852  
853  
854  
855  
856  
857  
858  
859  
859  
860  
861  
862  
863  
864  
865  
866  
867  
868  
869  
869  
870  
871  
872  
873  
874  
875  
876  
877  
878  
879  
879  
880  
881  
882  
883  
884  
885  
886  
887  
888  
889  
889  
890  
891  
892  
893  
894  
895  
896  
897  
898  
899  
900  
901  
902  
903  
904  
905  
906  
907  
908  
909  
909  
910  
911  
912  
913  
914  
915  
916  
917  
918  
919  
919  
920  
921  
922  
923  
924  
925  
926  
927  
928  
929  
929  
930  
931  
932  
933  
934  
935  
936  
937  
938  
939  
939  
940  
941  
942  
943  
944  
945  
946  
947  
948  
949  
949  
950  
951  
952  
953  
954  
955  
956  
957  
958  
959  
959  
960  
961  
962  
963  
964  
965  
966  
967  
968  
969  
969  
970  
971  
972  
973  
974  
975  
976  
977  
978  
979  
979  
980  
981  
982  
983  
984  
985  
986  
987  
988  
989  
989  
990  
991  
992  
993  
994  
995  
996  
997  
998  
999  
1000  
1001  
1002  
1003  
1004  
1005  
1006  
1007  
1008  
1009  
1009  
1010  
1011  
1012  
1013  
1014  
1015  
1016  
1017  
1018  
1019  
1019  
1020  
1021  
1022  
1023  
1024  
1025  
1026  
1027  
1028  
1029  
1029  
1030  
1031  
1032  
1033  
1034  
1035  
1036  
1037  
1038  
1039  
1039  
1040  
1041  
1042  
1043  
1044  
1045  
1046  
1047  
1048  
1049  
1049  
1050  
1051  
1052  
1053  
1054  
1055  
1056  
1057  
1058  
1059  
1059  
1060  
1061  
1062  
1063  
1064  
1065  
1066  
1067  
1068  
1069  
1069  
1070  
1071  
1072  
1073  
1074  
1075  
1076  
1077  
1078  
1079  
1079  
1080  
1081  
1082  
1083  
1084  
1085  
1086  
1087  
1088  
1089  
1089  
1090  
1091  
1092  
1093  
1094  
1095  
1096  
1097  
1098  
1099  
1099  
1100  
1101  
1102  
1103  
1104  
1105  
1106  
1107  
1108  
1109  
1109  
1110  
1111  
1112  
1113  
1114  
1115  
1116  
1117  
1118  
1119  
1119  
1120  
1121  
1122  
1123  
1124  
1125  
1126  
1127  
1128  
1129  
1129  
1130  
1131  
1132  
1133  
1134  
1135  
1136  
1137  
1138  
1139  
1139  
1140  
1141  
1142  
1143  
1144  
1145  
1146  
1147  
1148  
1149  
1149  
1150  
1151  
1152  
1153  
1154  
1155  
1156  
1157  
1158  
1159  
1159  
1160  
1161  
1162  
1163  
1164  
1165  
1166  
1167  
1168  
1169  
1169  
1170  
1171  
1172  
1173  
1174  
1175  
1176  
1177  
1178  
1179  
1179  
1180  
1181  
1182  
1183  
1184  
1185  
1186  
1187  
1188  
1189  
1189  
1190  
1191  
1192  
1193  
1194  
1195  
1196  
1197  
1198  
1198  
1199  
1199  
1200  
1201  
1202  
1203  
1204  
1205  
1206  
1207  
1208  
1209  
1209  
1210  
1211  
1212  
1213  
1214  
1215  
1216  
1217  
1218  
1219  
1219  
1220  
1221  
1222  
1223  
1224  
1225  
1226  
1227  
1228  
1229  
1229  
1230  
1231  
1232  
1233  
1234  
1235  
1236  
1237  
1238  
1239  
1239  
1240  
1241  
1242  
1243  
1244  
1245  
1246  
1247  
1248  
1249  
1249  
1250  
1251  
1252  
1253  
1254  
1255  
1256  
1257  
1258  
1259  
1259  
1260  
1261  
1262  
1263  
1264  
1265  
1266  
1267  
1268  
1269  
1269  
1270  
1271  
1272  
1273  
1274  
1275  
1276  
1277  
1278  
1279  
1279  
1280  
1281  
1282  
1283  
1284  
1285  
1286  
1287  
1288  
1289  
1289  
1290  
1291  
1292  
1293  
1294  
1295  
1296  
1297  
1298  
1298  
1299  
1299  
1300  
1301  
1302  
1303  
1304  
1305  
1306  
1307  
1308  
1309  
1309  
1310  
1311  
1312  
1313  
1314  
1315  
1316  
1317  
1318  
1319  
1319  
1320  
1321  
1322  
1323  
1324  
1325  
1326  
1327  
1328  
1329  
1329  
1330  
1331  
1332  
1333  
1334  
1335  
1336  
1337  
1338  
1339  
1339  
1340  
1341  
1342  
1343  
1344  
1345  
1346  
1347  
1348  
1349  
1349  
1350  
1351  
1352  
1353  
1354  
1355  
1356  
1357  
1358  
1359  
1359  
1360  
1361  
1362  
1363  
1364  
1365  
1366  
1367  
1368  
1369  
1369  
1370  
1371  
1372  
1373  
1374  
1375  
1376  
1377  
1378  
1379  
1379  
1380  
1381  
1382  
1383  
1384  
1385  
1386  
1387  
1388  
1389  
1389  
1390  
1391  
1392  
1393  
1394  
1395  
1396  
1397  
1398  
1398  
1399  
1399  
1400  
1401  
1402  
1403  
1404  
1405  
1406  
1407  
1408  
1409  
1409  
1410  
1411  
1412  
1413  
1414  
1415  
1416  
1417  
1418  
1419  
1419  
1420  
1421  
1422  
1423  
1424  
1425  
1426  
1427  
1428  
1429  
1429  
1430  
1431  
1432  
1433  
1434  
1435  
1436  
1437  
1438  
1439  
1439  
1440  
1441  
1442  
1443  
1444  
1445  
1446  
1447  
1448  
1449  
1449  
1450  
1451  
1452  
1453  
1454  
1455  
1456  
1457  
1458  
1459  
1459  
1460  
1461  
1462  
1463  
1464  
1465  
1466  
1467  
1468  
1469  
1469  
1470  
1471  
1472  
1473  
1474  
1475  
1476  
1477  
1478  
1479  
1479  
1480  
1481  
1482  
1483  
1484  
1485  
1486  
1487  
1488  
1489  
1489  
1490  
1491  
1492  
1493  
1494  
1495  
1496  
1497  
1498  
1498  
1499  
1499  
1500  
1501  
1502  
1503  
1504  
1505  
1506  
1507  
1508  
1509  
1509  
1510  
1511  
1512  
1513  
1514  
1515  
1516  
1517  
1518  
1519  
1519  
1520  
1521  
1522  
1523  
1524  
1525  
1526  
1527  
1528  
1529  
1529  
1530  
1531  
1532  
1533  
1534  
1535  
1536  
1537  
1538  
1539  
1539  
1540  
1541  
1542  
1543  
1544  
1545  
1546  
1547  
1548  
1549  
1549  
1550  
1551  
1552  
1553  
1554  
1555  
1556  
1557  
1558  
1559  
1559  
1560  
1561  
1562  
1563  
1564  
1565  
1566  
1567  
1568  
1569  
1569  
1570  
1571  
1572  
1573  
1574  
1575  
1576  
1577  
1578  
1579  
1579  
1580  
1581  
1582  
1583  
1584  
1585  
1586  
1587  
1588  
1589  
1589  
1590  
1591  
1592  
1593  
1594  
1595  
1596  
1597  
1598  
1598  
1599  
1599  
1600  
1601  
1602  
1603  
1604  
1605  
1606  
1607  
1608  
1609  
1609  
1610  
1611  
1612  
1613  
1614  
1615  
1616  
1617  
1618  
1619  
1619  
1620  
1621  
1622  
1623  
1624  
1625  
1626  
1627  
1628  
1629  
1629  
1630  
1631  
1632  
1633  
1634  
1635  
1636  
1637  
1638  
1639  
1639  
1640  
1641  
1642  
1643  
1644  
1645  
1646  
1647  
1648  
1649  
1649  
1650  
1651  
1652  
1653  
1654  
1655  
1656  
1657  
1658  
1659  
1659  
1660  
1661  
1662  
1663  
1664  
1665  
1666  
1667  
1668  
1669  
1669  
1670  
1671  
1672  
1673  
1674  
1675  
1676  
1677  
1678  
1679  
1679  
1680  
1681  
1682  
1683  
1684  
1685  
1686  
1687  
1688  
1689  
1689  
1690  
1691  
1692  
1693  
1694  
1695  
1696  
1697  
1698  
1698  
1699  
1699  
1700  
1701  
1702  
1703  
1704  
1705  
1706  
1707  
1708  
1709  
1709  
1710  
1711  
1712  
1713  
1714  
1715  
1716  
1717  
1718  
1719  
1719  
1720  
1721  
1722  
1723  
1724  
1725  
1726  
1727  
1728  
1729  
1

development, improvement of contrast, sensitization). Preferred examples of such compounds include polyalkylene oxides having a molecular weight of 600 or more as described in JP-B-58-9412 (the term "JP-B" as used herein means an "examined Japanese patent publication").

The photographic emulsion of the present invention may comprise a dispersion of a water-insoluble or sparingly soluble synthetic polymer for the purpose of improving dimensional stability. For example, alkyl (meth)acrylate, alkoxyalkyl (meth)acrylate, (meth)acrylamide, vinyl ester (e.g., vinyl acetate), acrylonitrile, and the like can be used, singly or in combination.

The emulsion to be used in the present invention may advantageously comprise as a protective colloid mainly gelatin, particularly inert gelatin. Besides gelatin, photographically inert gelatin derivatives (e.g., phthalated gelatin), and water-soluble synthetic polymers (e.g., polyvinyl acrylate, polyvinyl alcohol, polyvinyl pyrrolidone, dextran, polyacrylamide) can be used generally in an amount of 5 to 50 wt % based on the weight of gelatin. In particular, dextran and/or polyacrylamide can be used in combination with gelatin.

Plasticizers can also be added to the emulsion generally in an amount of 2 to 20 wt % based on the weight of the protective colloid in the emulsion, and polyols such as trimethylol propane, pentanediol, butanediol, ethylene glycol, and glycerin can be used for the purpose.

The material of the present invention may comprise any proper photographic support, such as glass or a film base (e.g., cellulose acetate, cellulose acetate butyrate, polyester (e.g., polyethylene terephthalate)). Preferably, the support is colored blue.

The surface of the support is preferably subjected to corona discharge treatment, glow discharge treatment, or ultraviolet-light irradiation treatment to improve the adhesion to the hydrophilic colloidal layer.

Alternatively, a subbing layer comprising a styrene-butadiene latex, vinylidene chloride latex, or the like may be provided on the support. A gelatin layer may be further provided on the subbing layer. As another alternative, a subbing layer comprising an organic solvent containing a polyethylene swelling agent and gelatin may be provided on the support.

These subbing layers may be further subjected to surface treatment to improve the adhesion to the hydrophilic colloidal layer.

The silver halide photographic material of the present invention can contain a developing agent such as hydroquinone, catechol, aminophenol, 3-pyrazolidone, ascorbic acid and derivatives thereof, reductone, and phenylenediamine. A combination of these developing agents can be used. The developing agent can be incorporated in the silver halide emulsion layer and/or other photographic layers (e.g., surface protective layer, interlayer, filter layer, antihalation layer, back layer). The developing agent can be incorporated in these layers in the form of solution in a suitable solvent or a dispersion as described in U.S. Pat. No. 2,592,368, and French Patent 1,505,778.

In the present invention, finely divided grains of organic compounds such as polymethyl methacrylate as described in U.S. Pat. Nos. 2,992,101, 2,701,245, 4,142,894, and 4,396,706, a polymer of methyl methacrylate with methacrylic acid and starch, or inorganic compounds such as silica, titanium dioxide, strontium sulfate and barium sulfate can be added as matting

agents in the protective layer (e.g., a surface protective layer). The amount of the matting agent is generally from 2 to 20 wt % based on the protective colloid in the protective layer. The grain size is preferably in the range of 1.0 to 10  $\mu\text{m}$ , particularly 2 to 5  $\mu\text{m}$ . In particular, a matting agent having a size of 0.3 to 1.3  $\mu\text{m}$  may be preferably used in an amount of 70 to 250 mg/m<sup>2</sup>.

A surface protective layer in the photographic light-sensitive material of the present invention may comprise as lubricant a silicone compound as described in U.S. Pat. Nos. 3,489,576 and 4,047,958 or colloidal silica as described in JP-B-56-23139. Besides these lubricants, parrafin wax, a higher aliphatic ester, and a starch derivative may be used.

The photographic processing of the photographic material prepared according to the present invention can be accomplished by any known method. As the processing solution, any known processing solution can be used. The processing temperature is normally between 18° C. and 50° C. Depending on the purpose, either development in which a silver image is formed (black-and-white photographic processing) or color photographic processing consisting of development in which a dye image is formed can be used. In particular, development can be accomplished by the method as described in *Research Disclosure* No. 17643, Vol. 176 (pp. 28-29) and No. 18716, Vol. 187 (from the left column to the right column on page 651).

In the ultrahigh speed processing of the present invention, the emulsion layer and/or other hydrophilic colloidal layers may preferably comprise an organic substance which can be eluted during development. If the substance to be eluted is gelatin, it is preferably a gelatin seed which does not take part in the crosslinking reaction of gelatin with a film hardener, such as acetylated gelatin and phthalated gelatin. Such a gelatin seed preferably has a small molecular weight. On the other hand, polyacrylamide as described in U.S. Pat. No. 3,271,158 and hydrophilic polymers such as polyvinyl alcohol and polyvinyl pyrrolidone can effectively be used as high molecular weight compounds other than gelatin. Saccharides such as dextran, saccharose and pullulan can also be effectively used. Preferred among these compounds are polyacrylamide and dextran. Particularly preferred among these compounds is polyacrylamide. These organic substances each preferably has an average molecular weight of 20,000 or less, preferably 10,000 or less.

Because of its excellent properties, a combination of dihydroxybenzene and 1-phenyl-3-pyrazolidone may be most preferably used as a black-and-white developer in the development step of the present invention. A p-aminophenol developing agent can also be used.

Examples of dihydroxybenzene developing agents to be used in the present invention include hydroquinone, chlorohydroquinone, bromohydroquinone, isopropylhydroquinone, methylhydroquinone, 2,3-dichlorohydroquinone, 2,5-dichlorohydroquinone, 2,3-dibromohydroquinone, and 2,5-dimethylhydroquinone. Particularly preferred among these compounds is hydroquinone.

Examples of p-aminophenol developing agents to be used in the present invention include N-methyl-p-aminophenol, p-aminophenol, N-(8-hydroxyethyl)-p-amino-phenol, N-(4-hydroxyphenyl)glycin, 2-methyl-p-amino-phenol, and p-benzylaminophenol. Particularly preferred among these compounds is N-methyl-p-aminophenol.

Examples of 3-pyrazolidone developing agents to be used in the present invention include 1-phenyl-3-pyrazolidone, 1-phenyl-4,4-dimethyl-3-pyrazolidone, 1-phenyl-4-methyl-4-hydroxymethyl-3-pyrazolidone, 1-phenyl-4,4-dihydroxymethyl-3-pyrazolidone, 1-phenyl-5-methyl-3-pyrazolidone, 1-p-aminophenyl-4,4-dimethyl-3-pyrazolidone, 1-p-tolyl-4,4-dimethyl-3-pyrazolidone, and 1-p-tolyl-4-methyl-4-hydroxymethyl-3-pyrazolidone.

In general, the developing agent is preferably used in an amount of 0.01 to 1.2 mol/l.

Examples of sulfites to be used as preservative in development include sodium sulfite, potassium sulfite, lithium sulfite, ammonium sulfite, sodium bisulfite, and potassium metabisulfite. Such sulfites may be preferably used in an amount of 0.2 mol/l or more, particularly 0.4 mol/l or more. The upper limit of the amount of sulfite to be used is preferably 2.5 mol/l.

The pH of the developer to be used in the development is preferably in the range of 9 to 13, more preferably 10 to 12.

Examples of alkaline agents to be used for the adjustment of pH include pH adjusters such as sodium hydroxide, potassium hydroxide, sodium carbonate, potassium carbonate, sodium tertiary phosphate and potassium tertiary phosphate.

The developer may also contain a buffer such as a borate as described in JP-A-62-186259, saccharose, acetoxime or 5-sulfosalicylic acid as described in JP-A-60-93433, a phosphate, or a carbonate.

The developer may further contain a dialdehyde film hardener or a bisulfite adduct thereof. Specific examples of such a compound include glutaraldehyde and bisulfite adducts thereof.

Examples of additives which can be used besides the above-mentioned components include development inhibitors (e.g., sodium bromide, potassium bromide, potassium iodide), organic solvents (e.g., ethylene glycol, diethylene glycol, triethylene glycol, dimethylformamide, methyl cellosolve, hexylene glycol, ethanol, methanol), and antifoggants such as mercapto compounds (e.g., 1-phenyl-5-mercaptotetrazole, sodium 2-mercaptopbenzimidazole-5-sulfonate), indazole compounds (e.g., 5-nitroindazole), and benztriazole compounds (e.g., 5-methylbenztriazole). If necessary, the developer may further contain a toner, a surface active agent, a defoaming agent, a water hardener, or an amino compound as described in JP-A-56-106244.

In the development process used in the present invention, the developer may contain a silver stain inhibitor such as a compound as described in JP-A-56-24347.

The developer used in the present invention may also contain an amino compound such as an alkanolamine as described in JP-A-56-106244.

Furthermore, the developer may contain compounds as described in L. F. A. Mason, *Photographic Processing Chemistry*, Focal Press, 1966, pp. 226-229, U.S. Pat. Nos. 2,193,015, and 2,592,364, and JP-A-48-64933.

The fixing solution to be used in the present invention is an aqueous solution containing a thiosulfate and having a pH value of 3.8 or more, preferably 4.2 to 7.0, more preferably 4.5 to 5.5.

As a fixing agent, sodium thiosulfate, ammonium thiosulfate, or the like can be used. Particularly preferred among these fixing agents is ammonium thiosulfate, in view of the fixing rate. The amount of the fixing agent to be used can be altered suitably. It is normally in the range of about 0.1 mol/l to about 6 mol/l.

The fixing solution may contain a water-soluble aluminum salt which acts as film hardener. Examples of such a water-soluble aluminum salt include aluminum chloride, aluminum sulfate, and potassium alum.

The fixing solution may contain tartaric acid, citric acid, gluconic acid or derivatives thereof, singly or in combination. Such a compound is effective when used in an amount of 0.005 mol, particularly 0.01 to 0.03 mol, per 1 of fixing solution.

The fixing solution may optionally contain a preservative such as sulfite or bisulfite, a pH buffer such as acetic acid or boric acid, a pH adjustor such as sulfuric acid, a chelating agent capable of softening water, or compound as described in JP-A-62-78551.

In the ultrahigh speed processing of the present invention, the percent swelling of the photographic material is reduced (preferably to 100% to 200%) so that the effect of film hardening can be reduced. In particular, the effect of film hardening during development may be preferably made difficult so that the effect of film hardening during fixing can also be made difficult. To this end, the degree of swelling of the light-sensitive material may be reduced. The pH value of the fixing solution may be adjusted to 4.6 or more so that the film hardening reaction can be minimized. Alternatively, the fixing solution may be free of film hardener. The term "percent swelling" used herein means the ratio (in percent) of a total thickness of photographic layers of the photographic material after immersing in water at 21° C. for 30 one minute to that of the photographic material before immersing.

In the development process used in the present invention, the silver halide photographic material which has been developed and fixed can then be processed with a rinsing solution or stabilizing solution at a replenishment rate of 3 or less (including no replenishment, i.e., reservoir rinse) per m<sup>2</sup> of the photographic material.

In other words, the process used in the present invention not only enables water-saving processing but also eliminates the need for piping in the automatic developing machine.

As means for reducing the replenishment rate a multi-stage countercurrent process (e.g., two or three stages) has been used. The multi-stage countercurrent process can be applied to the present invention to effect washing at a higher efficiency because the photographic material which has been fixed is sequentially processed while being brought into contact with the processing solution towards the highest purity, i.e., no contamination with the fixing solution.

In the above mentioned water-saving processing or pipeless processing, the rinsing solution or stabilizing solution may be preferably subjected to anti-mold treatment.

Examples of anti-mold treatments which can be used in the present invention include an ultravioletlight irradiation process as described in JP-A-60-263939, a method utilizing a magnetic field as described in JP-A-60-263940, a method which comprises the use of an ion exchange resin to purify water as described in JP-A-61-131632, and a method utilizing a germicide as described in JP-A-62-115154, JP-A-62-153952 and JP-A-62-209532.

Furthermore, in combination with these additives, germicides, anti-mold agents, and surface active agents as described in L. E. West, "Water Quality Criteria", *Photo. Sci. & Eng.*, Vol. 9, No. 6 (1965), M. W. Beach, "Microbiological Growth in Motion-Picture Process-

ing", SMPTE Journal, Vol. 85 (1976), R.O. Deegan, "Photo Processing Wash Water Biocides", *J. Imaging Tech*, Vol. 10, No. 6 (1984), and JP-A-57-8542, JP-A-57-58143, JP-A-58-105145, JP-A-57-132146, JP-A-58-18631, JP-A-57-97530, and JP-A-57-157244 can be used.

The rinse bath or stabilizing bath may further contain as a microbiocide an isothiazoline compound as described in R. T. Kreiman, *J. Image. Tech*, Vol. 10, No. 6, p. 242 (1984), and *Research Disclosure* Nos. 20526, (May, 1981) and 22845 (Apr., 1983), or a compound as described in JP-A-62-209532.

The rinse bath or stabilizing bath may further contain a compound as described in Hiroshi Horiguchi, *Bokin Bobai no Kagaku*, Sankyo Shuppan, 1972, and Nihon Bokin Bobai Gakkai, *Bokin Bobai Gijutsu Handbook*, Hakuhodo, 1986.

In the present invention, if a small amount of a rinsing solution is used at the rinse step, a squeeze roller rinse bath as described in JP-A-62-32460 may be preferably provided.

The overflow solution from the rinse bath or stabilizing bath produced by replenishing these baths with water which has been subjected to anti-mold treatment may be partially or entirely used as a processing solution having a fixing capacity at the previous step as described in JP-A-60-235133.

The silver halide photographic material of the present invention is characterized in that when it is processed by an automatic developing machine which performs at least development, fixing, rinsing (or stabilizing) and drying, the conventional rapid processing is completed within 90 seconds from development to drying, while the ultrahigh speed processing is completed within 60 seconds from development to drying, i.e., between the point at which the tip of the photographic material begins to be dipped in the developer and the point at which the tip of the photographic material comes out from the drying zone after passing through the fixing, rinsing (or stabilizing) and drying steps (the so-called "dry-to-dry time").

Thus, unprecedently high speed processing can be effectively accomplished without adversely affecting other properties (picture quality) by using the photographic material of the present invention.

In the present invention, the term "development time" as used herein means the time between the point at which the tip of the photographic material to be processed is dipped in the developing tank solution and the point at which it is dipped in the following fixing solution in the automatic developing machine. The term "fixing time" as used herein means the time between the point at which the tip of the photographic material is dipped in the fixing tank solution and the point at which it is dipped in the following rinse tank solution (stabilizing solution). The term "rinse time" as used herein means the time during which the photographic material is dipped in the rinse tank solution.

The term "drying time" as used herein means the time during which the photographic material is in a drying zone in which it is dried with hot air at a temperature of 35° C. to 100° C., preferably 40° C. to 80° C.

In order to accomplish the ultrahigh speed processing of the present invention within a dry-to-dry time of 60 seconds, the development preferably takes place at a temperature of about 25° C. to about 50° C. for 6 seconds to 20 seconds, more preferably at a temperature of 30° C. to 40° C. for 6 seconds to 15 seconds.

The fixing temperature and time are similar to the developing temperature and time, respectively. Specifically the fixing preferably takes place at a temperature of about 20° C. to about 50° C. for 6 seconds to 20 seconds, more preferably at a temperature of 30° C. to 40° C. for 6 seconds to 15 seconds.

The rinse or stabilization preferably takes place at a temperature of 0° C. to 50° C. for 6 seconds to 20 seconds, more preferably at a temperature of 30° C. to 40° C. for 6 seconds to 15 seconds.

In accordance with the process for the present invention, the photographic light-sensitive material which has been developed, fixed and rinsed (or stabilized) is then squeezed free of wash water, i.e., dried through squeeze rollers. The drying takes place at a temperature of about 40° C. to about 100° C. The drying time can be altered accordingly based on the ambient condition.

The silver halide emulsion of the present invention can be applied to various usages. Examples of such applications include various photographic light-sensitive materials for printing, such as duplicating, reproduction, and offset master materials, special photographic light-sensitive materials such as X-ray photographic, flash photographic, and electron ray photographic materials, and other photographic light-sensitive materials, such as general copying paper, micro copying paper, direct positive type color light-sensitive material, quick stabilized light-sensitive material, diffusion transfer light-sensitive material, color diffusion light-sensitive material, and light-sensitive material suitable for a combined developing and fixing bath.

The present invention will be further described in the following examples, but the present invention should not be construed as being limited thereto. All parts, percents, and ratios are by weight unless otherwise indicated.

## EXAMPLE

### 1. Preparation of silver halide emulsion of the present invention

#### i) Preparation of thioether emulsion

A thioether having the structural formula  $\text{HOCH}_2\text{CH}_2\text{SCH}_2\text{CH}_2\text{SCH}_2\text{CH}_2\text{OH}$  was added to a reaction vessel containing gelatin and potassium bromide which had been heated to a temperature of 55° C. in a proper amount. An aqueous solution of silver nitrate and an aqueous solution of potassium bromide were then added to the system by a controlled double jet process while the pAg value of the system was kept at 7.6 to form grains. The amount of the thioether added was adjusted accordingly to control the average grain size to 0.42  $\mu\text{m}$ . The grains were cubic and monodisperse such that 98% of all the grains fell within  $\pm 40\%$  from the average grain size. The emulsion was then desalinated. Gelatin and 30,000 ppm of phenoxy ethanol as preservative were added to the emulsion so that the pH and pAg values thereof were adjusted to 6.8 and 8.9, respectively. Thiourea dioxide and chloroauric acid were added to the emulsion in amounts of 4 mg/mol Ag and 3.2 mg/mol Ag, respectively. The emulsion was then heated to a temperature of 65° C. for 80 minutes to form fogged nuclei. 1,000 g of the starting emulsion contained 111 g of silver and 35 g of gelatin. 2. Preparation of emulsion coating solution

1,000 g of the thus obtained emulsion were weighed out. Gelatin was added to the emulsion in the necessary amount as set forth below. The emulsion was then

heated to a temperature of 40° C. so that dissolution was made. To the emulsion were added 50 cc of a 0.8% methanol solution of 5-ethoxycarbonyl-1,3,3-trimethyl-2-[2-(2,4-dimethyl-9-oxopyrazolo[5,1-b]quinazoline-3-yl)vinyl]-3H-indolium-4-methylbenzene sulfonate as a 5 sensitizer, 20 cc of a 50 wt % aqueous solution of trimethylolpropane as a wetting agent, an aqueous solution of 4-hydroxy-6-methyl-1,3,3a,7-tetraazaindene as a stabilizer, an aqueous solution of dedecylbenzenesulfonate as a coating aid, an aqueous solution of polyacrylamide as a binding aid, and an aqueous solution of polypotassium-p-vinylbenzenesulfonate as a thickening 10 agent.

The necessary amount of gelatin added was the value required to give a desired coated amount of gelatin 15 when the coated amount of silver in the emulsion layer of the coated product was 2.6 g/m<sup>2</sup>. The necessary amount of gelatin added to each emulsion coating solution prepared for this Example is set forth below.

20

|                              |                                      |
|------------------------------|--------------------------------------|
| Emulsion Coating Solution a: | the added amount of gelatin was 0 g  |
| Emulsion Coating Solution b: | the added amount of gelatin was 51 g |
| Emulsion Coating Solution c: | the added amount of gelatin was 30 g |
| Emulsion Coating Solution d: | the added amount of gelatin was 64 g |
| Emulsion Coating Solution e: | the added amount of gelatin was 38 g |

30

### 3. Preparation of coating solution for protective layer in the light-sensitive material

To a 10 wt % aqueous solution of gelatin which had been heated to a temperature of 40° C. were added 10 cc of a 2 wt % aqueous solution of sodium polystyrene sulfonate as a thickening agent, two kinds of finely divided polymethyl methacrylate grains (1 g of grains with an average grain size of 2  $\mu$ m and 5 g of grains with an average grain size of 0.8  $\mu$ m) as a matting agent, a 4 wt % aqueous solution of N,N'-ethylenebis(vinylsulfonylacetamide) as a film hardener, an aqueous solution of sodium t-octylphenoxyethoxyethanesulfonate as a coating aid, an aqueous solution of polyethylene surface active agent of the following structural formulas (1)-(3) and an aqueous solution of a fluorine-containing compound of the following structural formula (4) as antistatic agents, 50 cc of a 15% aqueous solution of polyacrylamide, polyacrylic acid, and silica. Water was then added to the emulsion to make 15 l. Each of the protective layer coating solutions set forth below were prepared in this manner.

The content of the film hardener was adjusted to 1.5 wt % based on the total layer amount of gelatin in the protective layer and the emulsion layer so that the water swelling at 20° C. was 150%. Antistatic Agents:



60



65



65

-continued

(4)

By altering the amount of the 10 wt % aqueous solution of gelatin added during the preparation of the protective layer coating solution, the coated amount of gelatin in the protective layer in the coated product was altered.

| Protective Layer      |                                                              |
|-----------------------|--------------------------------------------------------------|
| Coating Solution i:   | made from 1,200 g of the 10 wt % aqueous solution of gelatin |
| Coating Solution ii:  | made from 1,500 g of the 10 wt % aqueous solution of gelatin |
| Coating Solution iii: | made from 2,000 g of the 10 wt % aqueous solution of gelatin |
| Coating Solution iv:  | made from 2,200 g of the 10 wt % aqueous solution of gelatin |
| Coating Solution v:   | made from 2,500 g of the 10 wt % aqueous solution of gelatin |
| Coating Solution vi:  | made from 2,700 g of the 10 wt % aqueous solution of gelatin |

### 4. Preparation of back coating solution

To 1,000 g of a 10 wt % aqueous solution of gelatin which had been heated to a temperature of 40° C. were 35 added an aqueous solution of sodium polyethylene sulfonate as a thickening agent, 400 cc of each of 6% an aqueous solution containing 6% of each of dyes having the following structural formulae (5)-(7), an aqueous solution of N,N'-ethylenebis-(vinylsulfonylacetamide) 40 as a film hardener, an aqueous solution of sodium t-octylphenoxyethoxyethanesulfonate as a coating aid, finely divided polymethyl methacrylate grains (average grain size: 1.2  $\mu$ m), silica, and an aqueous solution of a copolymer of methyl methacrylate and ethyl acrylate. 45 Thus, a back coating solution as prepared.

#### Dyes



(5)



(6)

-continued

Dyes

## 5. Preparation of coating solution of surface protective layer for back layer

To a 10 wt % aqueous solution of gelatin which had been heated to a temperature of 40° C. were added an aqueous solution of sodium polystyrenesulfonate as thickening agent, finely divided polymethylmethacrylate grains (average grain size: 3.0  $\mu\text{m}$ ) as matting agent, an aqueous solution of sodium t-octylphenoxyethoxyethanesulfonate as coating aid, and an aqueous solution of polyethylene surface active agents of the structural formulas (2) and (3) described above and an aqueous solution of a fluorine-containing of the following formulas (8)–(10) as antistatic agents compound to prepare a coating solution. Antistatic Agents:



## 6. Preparation of coated specimens

The above mentioned back coating solution and back protective layer coating solution were coated together on one side of a polyethylene terephthalate support in amounts such that the gelatin content of the back layer and the back protective layer reached 2.5  $\text{g/m}^2$  and 1  $\text{g/m}^2$ , respectively, thereby totalling 3.5  $\text{g/m}^2$ .

The emulsion coating solution as prepared in section 2 and the protective layer coating solution as prepared in section 3 were then added to the other side of support in that order. The coated amount of gelatin in the emulsion layer and the protective layer was according the combinations as set forth below. The coated amount of silver was adjusted to 2.6  $\text{g/m}^2$ .

- Coated specimen I: prepared from Emulsion Coating Solution a and Protective Layer Coating Solution ii, with the coated amounts of gelatin being 1  $\text{g/m}^2$  and 1.5  $\text{g/m}^2$ , respectively, thereby totalling 2.5  $\text{g/m}^2$
- Coated specimen II: prepared from Emulsion Coating Solution a and Protective Layer Coating Solution v, with the coated amounts of gelatin being 1  $\text{g/m}^2$  and 2.5  $\text{g/m}^2$ , respectively, thereby totalling 3.5  $\text{g/m}^2$
- Coated specimen III: prepared from Emulsion Coating Solution b and Protective Layer Coating Solution ii, with the coated amounts of gelatin being 2.0  $\text{g/m}^2$  and 1.5  $\text{g/m}^2$ , respectively, thereby totalling 3.5  $\text{g/m}^2$
- Coated specimen IV: prepared from Emulsion Coating

12

-continued

|     |    |                                                                                                                                                                                                                                                                                                                                                                                                                                                |
|-----|----|------------------------------------------------------------------------------------------------------------------------------------------------------------------------------------------------------------------------------------------------------------------------------------------------------------------------------------------------------------------------------------------------------------------------------------------------|
| (7) | 5  | Solution c and Protective Layer Coating Solution iii, with the coated amounts of gelatin being 1.5 $\text{g/m}^2$ and 2.0 $\text{g/m}^2$ , respectively, thereby totalling 3.5 $\text{g/m}^2$<br>Coated specimen a: prepared from Emulsion Coating Solution a and Protective Layer Coating Solution i, with the coated amounts of gelatin being 1.0 $\text{g/m}^2$ and 1.2 $\text{g/m}^2$ , respectively, thereby totalling 2.2 $\text{g/m}^2$ |
|     | 10 | Coated specimen b: prepared from Emulsion Coating Solution a and Protective Layer Coating Solution vi, with the coated amounts of gelatin being 0.8 $\text{g/m}^2$ and 2.7 $\text{g/m}^2$ , respectively, thereby totalling 3.5 $\text{g/m}^2$                                                                                                                                                                                                 |
|     | 15 | Coated specimen c: prepared from Emulsion Coating Solution d and Protective Layer Coating Solution ii, with the coated amounts of gelatin being 2.3 $\text{g/m}^2$ and 1.5 $\text{g/m}^2$ , respectively, thereby totalling 3.8 $\text{g/m}^2$                                                                                                                                                                                                 |
|     | 20 | Coated specimen d: prepared from Emulsion Coating Solution e and Protective Layer Coating Solution iv, with the coated amounts of gelatin being 1.7 $\text{g/m}^2$ and 2.2 $\text{g/m}^2$ , respectively, thereby totalling 3.9 $\text{g/m}^2$                                                                                                                                                                                                 |
|     | 25 | Coated specimen e: prepared from Emulsion Coating Solution d and Protective Layer Coating Solution i, with the coated amounts of gelatin being 2.3 $\text{g/m}^2$ and 1.2 $\text{g/m}^2$ , respectively, thereby totalling 3.5 $\text{g/m}^2$                                                                                                                                                                                                  |
|     | 30 |                                                                                                                                                                                                                                                                                                                                                                                                                                                |

These coated specimens were stored at a temperature of 20° C. and a relative humidity of 65% for 7 days, and then evaluated for the following properties.

## 7. Evaluation of dryability

The coated specimens were uniformly exposed to light from a BLB light source (emitting light having a peak at a wavelength of 365 nm) at room temperature for 15 seconds in a duplicator available from Du Pont. These specimens were then subjected to 45-second speed processing with a developer RD-7 (a product of Fuji Photo Film Co., Ltd.) and a fixing solution Fuji F (a product of Fuji Photo Film Co., Ltd.) at a temperature of 35° C. in an automatic developing machine (manufactured by Fuji Photo Film Co., Ltd.). 30 sheets (35.6 cm  $\times$  43.2 cm) of these specimens were continuously processed to reach the steady state of processings. If the 30th sheet was dry, the specimen was considered to pass the dryability test (P). On the other hand, if the 30th sheet was not yet dry, the specimen was considered to fail the test (F).

## 8. Evaluation of roller marking

The coated specimens were uniformly exposed to light from a BLB light source in a duplicator available from Du Pont at room temperature in such a manner that the optical density after processing was about 1.0. The specimens were then processed with Developer RD-7 and Fixing Solution Fuji F in the automatic developing machine FPM-9000 at a temperature of 35° C. Each specimen was then examined for roller marks. If 65 roller marks were discovered, the specimen was considered to fail the test (F). On the other hand, if no roller marks were discovered, the specimen was considered to pass the test (P).

## 9. Evaluation of scratch pinholing

Film specimens (35.6 cm  $\times$  43.2 cm) which had not been exposed were processed with Developer RD-7 5 and Fixing Solution Fuji F in the automatic developing machine FPM-9000 at a temperature of 35° C. These film specimens were mounted on a ground glass plate under which lamps were placed. The system was 10 screened from external light. The room lamp was then turned off. The pinholes were then counted. If 50 or more pinholes were counted, the specimen was considered to fail the test (F). On the other hand, if less than 50 15 pinholes were counted, the specimen was considered to pass the test (P).

## 10. Results

The results from the evaluations are set forth below in Table 1.

Only the specimens of the present invention passed all of the tests.

TABLE 1

| Coat<br>Speci-<br>men | Coated amount of<br>gelatin (g/m <sup>2</sup> ) |                          |            | Judgement of<br>properties |                     |                    | Overall<br>judge-<br>ment |
|-----------------------|-------------------------------------------------|--------------------------|------------|----------------------------|---------------------|--------------------|---------------------------|
|                       | Emul-<br>sion<br>layer                          | Protec-<br>tive<br>layer | To-<br>tal | Dry-<br>abil-<br>ity       | Roll-<br>er<br>mark | Scratch<br>pinhole |                           |
| I                     | 1.0                                             | 1.5                      | 2.5        | P                          | P                   | P                  | P                         |
| II                    | 1.0                                             | 2.5                      | 3.5        | P                          | P                   | P                  | P                         |
| III                   | 2.0                                             | 1.5                      | 3.5        | P                          | P                   | P                  | P                         |
| IV                    | 1.5                                             | 2.0                      | 3.5        | P                          | P                   | P                  | P                         |

TABLE 1-continued

| Coat<br>Speci-<br>men | Coated amount of<br>gelatin (g/m <sup>2</sup> ) |                          |            | Judgement of<br>properties |                     |                    | Overall<br>judge-<br>ment |
|-----------------------|-------------------------------------------------|--------------------------|------------|----------------------------|---------------------|--------------------|---------------------------|
|                       | Emul-<br>sion<br>layer                          | Protec-<br>tive<br>layer | To-<br>tal | Dry-<br>abil-<br>ity       | Roll-<br>er<br>mark | Scratch<br>pinhole |                           |
| a                     | 1.0                                             | 1.2                      | 2.2        | P                          | P                   | F                  | F                         |
| b                     | 0.8                                             | 2.7                      | 3.5        | P                          | F                   | P                  | F                         |
| c                     | 2.5                                             | 1.5                      | 3.8        | F                          | P                   | P                  | F                         |
| d                     | 1.7                                             | 2.2                      | 3.9        | F                          | P                   | P                  | F                         |
| e                     | 2.3                                             | 1.2                      | 3.5        | P                          | P                   | F                  | F                         |

(Note: Specimens I, II, III, and IV were in accordance with the present invention, while the other specimens were comparative)

While the invention has been described in detail and with reference to specific embodiments thereof, it will be apparent to one skilled in the art that various changes and modifications can be made therein without departing from the spirit and scope thereof.

## What is claimed is:

- 20 1. A silver halide photographic material element comprising a support having thereon, in sequence, a hydrophilic silver halide emulsion layer and a protective layer, wherein gelatin is contained in said protective layer in an amount of at least 1.5 g/m<sup>2</sup>, gelatin is contained in said emulsion layer in an amount of at least 1.0 g/m<sup>2</sup>, and the coated amount of gelatin in said protective layer and said emulsion layer is a total of at most 3.5 g/m<sup>2</sup>.
- 25 2. A silver halide photographic material element as in claim 1, wherein said gelatin is inert gelatin.
- 30 3. A silver halide photographic material element as in claim 1, wherein at least one of dextran and polyacrylamide is present together with gelatin in said emulsion layer.
- 35 4. A silver halide photographic material element as in claim 1, wherein said support is colored blue.

\* \* \* \* \*